

## UNITED STATES PATENT OFFICE

2,057,960

## FIBER TREATING COMPOSITION

Leroy A. Kramer, Chicago, Ill., assignor to Victor Chemical Works, a corporation of Illinois

No Drawing. Application November 14, 1935,  
Serial No. 49,823

3 Claims. (Cl. 134—15)

This application relates to a fiber treating composition, and particularly to a water-proofing and water-repelling fiber treating composition.

The use of waxes as a water-repellent material 5 has been known for some time, and certain emulsions of wax have also been suggested. In some instances, such emulsions have been stabilized by the addition of aluminum salts and colloidal materials such as glue or gelatine, the aluminum salt, 10 generally the acetate, acting as an electronic or stabilizing agent.

It has now been discovered that a casein solution, such as is produced by the process described in U. S. application, Serial No. 13,785 of Hans B. 15 Gottlieb, may be made more water repellent by the addition of small amounts of waxes, and that a stable emulsion may be produced with such a compound without the addition of a stabilizing salt.

20 The compound described in the Gottlieb application may be prepared by the solution of casein in a minor proportion of aluminum formate. The preferred mixture comprises 30 parts of aluminum formate and 70 parts of casein, which are 25 introduced into approximately 600 parts of hot water at 75 to 80° C. and held at this temperature for approximately 20 minutes to effect solution of the aluminum formate, after which the temperature is lowered to about 55 to 60° C. and 30 there maintained until the casein is completely dissolved.

The amount of aluminum formate may be varied from 10 to 50% and the casein from 50 to 35, preferably the aluminum formate is within 35 the range of 25 to 35%. The reaction product produced contains both aluminum and casein in the molecule, but its exact structure is not understood.

40 This casein aluminum formate complex is not appreciably hydrolyzed by water, and has excellent water-proofing characteristics when applied to a fibrous material. Its water repellence, however, may be improved by the addition of a wax.

45 A stable wax emulsion may be produced from the above described product without the presence of aluminum salt, by the simple addition of a wax, such as bees-wax, petroleum jelly, carnauba wax, paraffin and the like, and its emulsification 50 with the caseinous reaction product in any suitable manner.

A preferred manner of emulsifying the product consists in the agitation of an aqueous solution 55 of caseinous material with wax and a partial wax solvent. For example, the solution produced

from 70 parts casein, 30 parts aluminum formate and 600 parts of hot water is rapidly agitated while adding a homogeneous mixture of 100 parts paraffin, 15 parts tetralin and 15 parts hexalin. Under agitation this becomes emulsified to produce a stable jelly-like product which may be diluted with warm water and used as a bath for treating paper, cotton or wool fabrics. 5

Normally, a dilution equivalent to 1 to 5% of non-aqueous constituents is used. The fabric to 10 be treated is held in the bath at a temperature of about 60° C. for a few minutes, removed, and the excess emulsion drained off and squeezed off between a pair of rolls. The fabric may then be dried at a temperature of the order of 60° C. A 15 fabric so treated is pliable and soft and does not have a waxy feel. It is fully water-proof and water-repellent.

The above emulsion may be used in much more dilute concentration than other wax emulsions. 20 Thus, the actual wax concentration may range from only about one-half to two and one-half percent. The emulsion will remain in stable form for periods of 24 hours or more at temperatures of the order of 60° C. The wax is emulsified in 25 extremely fine particle size which permits the even distribution of a much thinner film on the fibers of the fabric than has heretofore been possible in a single stage water-proofing and water-repellent process. 30

If desired, odor-masking agents such as pine-oil, terpineol, or the like may be introduced into the emulsion to disguise any disagreeable odor due to the casein.

35 It is much preferred to use a partial solvent material or emulsifying agent such as tetralin or hexalin, but it is possible to secure a very satisfactory composition without these agents.

The foregoing detailed description has been given for clearness of understanding only, and no 40 unnecessary limitations should be understood therefrom, but the appended claims should be construed as broadly as permissible, in view of the prior art.

45 I claim:

1. A stable fiber treating emulsion comprising a wax and an aqueous solution of a reaction product of casein and aluminum formate such reaction product having no free aluminum ions.

2. A stable fiber treating emulsion comprising 50 a wax and an aqueous solution of a reaction product of casein and aluminum formate such reaction product having no free aluminum ions and a partial solvent for the wax.

3. A composition as set forth in claim 2, in 55

which the partial solvent is a compound of the class consisting of tetratin and hexalin.

4. A composition of matter comprising approximately equal parts of a wax and a caseinous reaction product of casein and aluminum formate such reaction product having no free aluminum ions, a relatively large amount of water and a small amount of a partial solvent for the wax.

5. An emulsion comprising approximately 100 parts of paraffin, 15 parts of tetratin, 15 parts of hexalin, 100 parts of a casein aluminum formate reaction product such reaction product having no free aluminum ions, and 600 parts of water.

6. A stable fiber treating emulsion comprising

an aqueous emulsion of a wax and an aqueous solution of the reaction product of casein and aluminum formate, said reaction product having no free aluminum ions, the proportion of wax being approximately .5 to 2.5% of the emulsion. 5

7. An emulsion as set forth in claim 6, in which the wax and the caseinous reaction product are present in approximately equal proportions.

8. A stable fiber treating emulsion comprising a wax and an aqueous solution of a reaction product of casein and aluminum formate, such reaction product having 25 to 35 parts of aluminum formate combined with 75 to 65 parts of casein. 10

LEROY A. KRAMER.